

## UNITED STATES PATENT OFFICE

2,410,021

## FLOTATION PROCESS

Fred D. De Vaney, Hibbing, Minn., assignor to  
 Erie Mining Company, Hibbing, Minn., a corporation of Minnesota

No Drawing. Application April 26, 1944,  
 Serial No. 532,867

10 Claims. (Cl. 209—166)

1

This invention relates to specific improvements in the froth floatative beneficiation of silicious iron ores, and is specifically concerned with a mode of accelerating the rate of floatative separation of silicious gangue from such ores using higher molecular weight aliphatic amine compounds as cationic collectors.

It heretofore has been suggested that silicious iron ores might be beneficiated by froth-floating the silicious gangue particles from the iron mineral particles of a pulp of the ore by the use of a higher molecular weight aliphatic amine compound, having from 10 to 18 carbon atoms in the aliphatic radical, as collector in conjunction with a suitable frother. According to the suggested technique the pulp circuit was to be maintained distinctly alkaline; preferably, also, the flotation was to be effected in the presence of a selectivity-improving agent such as acid-treated starch.

2

the ore pulp a relatively small amount of an alkali metal sulfide (specifically, sodium sulfide), the rate of floatation of the silicious gangue particles can be very materially increased, with no decrease in the selectivity and with a small but appreciable saving in the amount of amine collector required. As equivalent of sodium sulfide there may be used potassium sulfide or calcium sulfide or barium sulfide or a polysulfide of sodium, potassium, calcium or barium.

It has been found that the alkali metal or alkaline earth metal sulfide or polysulfide functions most effectively when the pulp circuit is maintained acid (i. e., less than pH 7) rather than alkaline.

The influence of progressive additions of sodium sulfide, while maintaining a constant pH, may be seen from the data of the following table:

TABLE 1  
*Effect of sodium sulfide on amine flotation of  
 Mesabi washing plant tailings*

| Amt.<br>sodium<br>sulfide,<br>lbs./ton<br>ore | Product              | Percent<br>wt. | Assay,<br>percent |        | Percent<br>total<br>iron | Total flotation<br>time |
|-----------------------------------------------|----------------------|----------------|-------------------|--------|--------------------------|-------------------------|
|                                               |                      |                | Iron              | Silica |                          |                         |
| None.....                                     | Silicious froth..... | 82.41          | 8.95              | -----  | 41.01                    | 4 min., 25 sec.         |
|                                               | Concentrate.....     | 17.59          | 60.24             | 8.15   | 58.99                    |                         |
|                                               | Total.....           | 100.00         | 17.97             | -----  | 100.00                   |                         |
|                                               | Silicious froth..... | 82.86          | 8.85              | -----  | 41.36                    | 4 min.                  |
|                                               | Concentrate.....     | 17.14          | 60.61             | 8.02   | 58.64                    |                         |
|                                               | Total.....           | 100.00         | 17.72             | -----  | 100.00                   |                         |
| 0.2.....                                      | Silicious froth..... | 82.48          | 8.63              | -----  | 39.92                    | 3 min., 25 sec.         |
|                                               | Concentrate.....     | 17.52          | 61.21             | 7.17   | 60.08                    |                         |
|                                               | Total.....           | 100.00         | 17.84             | -----  | 100.00                   |                         |
|                                               | Silicious froth..... | 83.66          | 9.61              | -----  | 44.42                    | 3 min.                  |
|                                               | Concentrate.....     | 16.34          | 61.54             | 6.60   | 55.58                    |                         |
|                                               | Total.....           | 100.00         | 18.10             | -----  | 100.00                   |                         |
| 0.8.....                                      | Silicious froth..... | 84.50          | 9.93              | -----  | 47.54                    | 2 min., 35 sec.         |
|                                               | Concentrate.....     | 15.50          | 59.75             | 9.34   | 52.46                    |                         |
|                                               | Total.....           | 100.00         | 17.65             | -----  | 100.00                   |                         |
|                                               | Silicious froth..... | 84.50          | 9.93              | -----  | 47.54                    | 2 min., 35 sec.         |
|                                               | Concentrate.....     | 15.50          | 59.75             | 9.34   | 52.46                    |                         |
|                                               | Total.....           | 100.00         | 17.65             | -----  | 100.00                   |                         |

*Note.*—In each test 500 gm. of washing plant tailing were treated without additional crushing and without desliming in a 500 gram Denver Sub A flotation cell. The pulp in each case was maintained at an acidity of pH 5.2. The flotation reagents used in each test were identical and consisted of 0.4 lb./ton of "AM Coco," i. e., a cationically-acting collector consisting of the hydrochlorides, acetates or other water-soluble forms of mixed primary aliphatic amines corresponding in aliphatic chain length to fatty acids of coconut oil, made by Armour & Company and .104 lb./ton of methyl amyl alcohol which were added in small increments. When sodium sulfide was used this reagent was conditioned with the pulp for 5 minutes prior to flotation.

It has now been found that if with the usual higher molecular weight aliphatic amine collector aforesaid and suitable frother there be added to

The influence of varying the acidity of the pulp circuit, while maintaining constant the amount of sodium sulfide (and all other variables) at

arbitrary levels, may be seen from the data of the following table:

TABLE 2  
*Effect of varying pH of pulp on amine flotation of Mesabi washing plant tailings*

| pH of pulp | Product         | Percent wt. | Assay, percent |        | Percent total iron | Total flotation time |
|------------|-----------------|-------------|----------------|--------|--------------------|----------------------|
|            |                 |             | Iron           | Silica |                    |                      |
| 6.0        | Silicious froth | 80.90       | 7.99           | -----  | 36.54              | 3 min., 30 sec.      |
|            | Concentrate     | 19.10       | 58.72          | 9.79   | 63.46              |                      |
|            | Total           | 100.00      | 17.68          | -----  | 100.00             |                      |
| 7.1        | Silicious froth | 79.66       | 8.00           | -----  | 35.39              | 5 min.               |
|            | Concentrate     | 20.34       | 57.16          | 12.53  | 64.61              |                      |
|            | Total           | 100.00      | 18.00          | -----  | 100.00             |                      |
| 8.0        | Silicious froth | 78.73       | 7.51           | -----  | 33.28              | 5 min., 45 sec.      |
|            | Concentrate     | 21.27       | 55.69          | 14.61  | 66.72              |                      |
|            | Total           | 100.00      | 17.76          | -----  | 100.00             |                      |

Test conditions same as given in Table 1, except 0.5# fused sodium sulfide used in all tests and alkalinity and acidity controlled by addition of either sulphuric acid or sodium carbonate.

By using in the pulp circuit both the sulfide and the acid-treated starch it is possible to maintain the high selectivity attributable to the use of the starch material while simultaneously achieving the high rate of feed made possible by use of the sulfide.

#### EXAMPLE

The starting material was a washing plant tailing from the Danube mine, Minnesota, analyzing 16.66% Fe, mostly as hematite. The silicious gangue was mostly quartz. The material as obtained was essentially of a size through 48 mesh and was not further subdivided.

The starting material, without having been subjected to a desliming treatment, and in the form of an aqueous pulp of approximately 25% solids, was added to a mechanically agitated flotation cell, and to it were added 0.5 lb./ton of acid-treated starch, 1/4 lb./ton of sulfuric acid monohydrate, and 0.8 lb./ton of sodium sulfide in the form of 60% fused flake. After thorough mixing of these ingredients with the pulp and conditioning for 3 minutes, froth flotation was induced by the addition of 0.25 lb./ton of "AM Coco" collector and 0.05 lb./ton of "B-23" frother, both of which agents were added, in small increments, during the agitation and aeration of the pulp. After 1 minute 45 seconds, a first froth, constituting a finished tailing, was removed. Additional amounts of the collector (0.10 lb./ton) and the frother (0.025 lb./ton) were added, and after 1 minute and 30 seconds a second froth was removed. This second froth was a middling product which, in the continuous flotation process, would be retreated along with fresh feed.

The following results were obtained:

| Product                   | Per cent wt. | Per cent Fe | Per cent SiO <sub>2</sub> | Per cent total iron |
|---------------------------|--------------|-------------|---------------------------|---------------------|
| Silicious froth (tailing) | 60.24        | 5.71        | -----                     | 20.65               |
| 2d froth (middling)       | 23.62        | 13.86       | -----                     | 19.63               |
| Concentrate               | 16.14        | 61.65       | 7.45                      | 59.72               |
|                           | 100.00       | 16.66       | 7.45                      | 100.00              |

It is to be noted that the time required for the over-all flotation (both roughing and cleaning) was 3 minutes and 15 seconds, whereas in the absence of the sodium sulfide the normal flotation time is from 5 to 6 minutes. This greatly

increased rate of flotation means that a flotation plant would require approximately only 60% as

many flotation cells to handle the same tonnage per day provided the alkali metal sulfide, in acid circuit, expedient is employed.

Repetition of the above example, substituting the equivalent amount of potassium sulfide for the sodium sulfide, gives results almost identical with those above set out. Calcium sulfide and barium sulfide have been substituted by me for the sodium or potassium sulfide and found to be helpful in accelerating the rate of flotation separation.

The accelerated flotation rate achieved when alkali metal or alkaline earth metal sulfide or polysulfide is used appears to be due to a selective flocculating effect of the sulfide or polysulfide on the gangue particles. Whatever may be the correct explanation, it is an observable fact that, with use of the sulfide or polysulfide, flocculation of the gangue particles does take place, and this flocculation of the gangue is definitely a very desirable condition for rapid flotation.

I have found that non-alkali inorganic sulfides such as ammonium sulfide and hydrogen sulfide not only do not serve to accelerate the rate of separating but positively are harmful in the flotation. A number of experiments with organic compounds of sulfur, e. g., petroleum sulfonates, sulfonic acids and a number of xanthates, have established that such compounds are not helpful for accelerating the rate of flotation.

It is to be noted, in this connection, that the function of the alkali metal or alkaline earth metal sulfide or polysulfide is not that of a sulfidizing agent toward the mineral to be floated, as obtains in the flotation of base metal ores, e. g., oxidized copper and lead ores, where a sulfide actually forms a base metal sulfide "sheath" or surface layer on the mineral particle. In the present process, no chemical combination between the silica and the sulfide or polysulfide of sodium, potassium, calcium or barium has been observed.

I claim:

1. In the process of beneficiating silicious iron ore by cationically froth-floating the silicious gangue particles from the iron mineral particles of an aqueous pulp of such an ore by the use of a higher molecular weight aliphatic amine collector and a frother, the step of accelerating the rate of flotation of the silicious gangue particles which consists in incorporating a relatively very small amount of sodium sulfide into the pulp prior to the froth flotation step.

2. In the process of beneficiating silicious iron

ore by cationically froth-floating the silicious gangue particles from the iron mineral particles of an aqueous pulp of such an ore by the use of a higher molecular weight aliphatic amine collector and a frother, the step of accelerating the rate of flotation of the silicious gangue particles which consists in maintaining the pulp at a pH of less than 7 but not less than about 5 and incorporating into the acidic pulp, prior to the froth flotation step, a relatively very small amount of sodium sulfide.

3. In the process of beneficiating silicious iron ore by froth floating the silicious gangue particles from the iron mineral particles of an aqueous pulp of such an ore using a higher molecular weight aliphatic amine as collector, a suitable frother, and acid-treated starch as selectivity-improving agent, steps of accelerating the rate of flotation of the silicious gangue particles which consists in maintaining the pulp containing the aforesaid agents at a pH of less than 7 but not less than about 5 and incorporating into the acidic pulp, prior to the froth flotation step, a relatively very small amount of sodium sulfide.

4. In the process of beneficiating silicious iron ore by cationically froth-floating the silicious gangue particles from the iron mineral particles of an aqueous pulp of such an ore by the use of a higher molecular weight aliphatic amine collector and a frother, the step of accelerating the rate of flotation of the silicious gangue particles which consists in incorporating a relatively very small amount of an alkali metal sulfide into the pulp prior to the froth flotation step.

5. In the process of beneficiating silicious iron ore by cationically froth-floating the silicious gangue particles from the iron mineral particles of an aqueous pulp of such an ore by the use of a higher molecular weight aliphatic amine collector and a frother, the step of accelerating the rate of flotation of the silicious gangue particles which consists in incorporating a relatively very small amount of an alkali metal polysulfide into the pulp prior to the froth flotation step.

6. In the process of beneficiating silicious iron ore by cationically froth-floating the silicious gangue particles from the iron mineral particles of an aqueous pulp of such an ore by the use of a higher molecular weight aliphatic amine collector and a frother, the step of accelerating the rate of flotation of the silicious gangue particles which consists in incorporating a relatively very small amount of a compound of the group consisting of the alkali metal sulfides, the alkaline earth metal sulfides, the alkali metal polysulfides and the alkaline earth metal polysulfides into the pulp prior to the froth flotation.

7. In the process of beneficiating silicious iron ore by cationically froth-floating the silicious gangue particles from the iron mineral particles of an aqueous pulp of such an ore by the use of a higher molecular weight aliphatic amine collector and of a frother, in a slightly acidic circuit, the step of selectively flocculating the silicious gangue particles which consists in incorporating into the pulp, prior to the flotation operation, a relatively small amount of a compound of the group consisting of the alkali metal sulfides, the alkaline earth metal sulfides, the alkali metal polysulfides and the alkaline earth metal polysulfides.

15 8. The process of beneficiating a silicious oxidic iron ore, which comprises adding to an aqueous pulp of the ore a mineral acid in an amount sufficient to give the pulp a pH of about 6.0, conditioning the pulp with from about 0.4 lb. to about 1.6 lbs./ton of a compound of the group consisting of alkali metal sulfides, alkaline earth metal sulfides, alkali metal polysulfides and alkaline earth metal polysulfides, and subjecting the acidified and conditioned pulp to froth flotation in the presence of a frother and of a higher molecular weight aliphatic amine collector, thereby rapidly raising a froth product rich in silicious gangue particles.

30 9. The process of beneficiating a silicious oxidic iron ore, which comprises adding to an aqueous pulp of the ore a mineral acid in an amount sufficient to give the pulp a pH of about 6.0, conditioning the pulp with acid-treated starch and from about 0.4 lb. to about 1.6 lbs./ton of a compound of the group consisting of alkali metal sulfides, alkaline earth metal sulfides, alkali metal polysulfides and alkaline earth metal polysulfides, and subjecting the acidified and conditioned pulp to froth flotation in the presence of a frother and of a higher molecular weight aliphatic amine collector, thereby rapidly raising a froth product rich in silicious gangue particles while depressing fine oxidic iron particles into the underflow product.

45 10. The process of beneficiating a silicious oxidic iron ore, which comprises adding to an aqueous pulp of the ore a mineral acid in an amount sufficient to give the pulp a pH of about 6.0, conditioning the pulp with from about 0.4 lb. to about 1.6 lbs./ton of sodium sulfide, and subjecting the acidified and conditioned pulp to froth flotation in the presence of a frother and of a primary alkylamine having from 10 to 18 carbon atoms in the alkyl radical as collector, thereby rapidly raising a froth product rich in silicious gangue particles.

FRED D. DE VANNEY.